

# United States Patent [19]

Shanton

[11] Patent Number: 4,509,065

[45] Date of Patent: Apr. 2, 1985

[54] RECORD MATERIAL

[75] Inventor: Kenneth J. Shanton, Beaconsfield, England

[73] Assignee: The Wiggins Teape Group Limited, Hampshire, England

[21] Appl. No.: 442,565

[22] Filed: Nov. 18, 1982

[30] Foreign Application Priority Data

Dec. 4, 1981 [GB] United Kingdom ..... 8136583  
Dec. 4, 1981 [GB] United Kingdom ..... 8136584  
Dec. 9, 1981 [GB] United Kingdom ..... 8137069  
Dec. 9, 1981 [GB] United Kingdom ..... 8137070  
Dec. 9, 1981 [GB] United Kingdom ..... 8137071  
Dec. 9, 1981 [GB] United Kingdom ..... 8137073

[51] Int. Cl.<sup>3</sup> ..... B41M 5/16; B41M 5/18;  
B41M 5/22

[52] U.S. Cl. ..... 346/225; 346/210;  
346/211; 346/212; 346/219; 346/226

[58] Field of Search ..... 282/27.5; 427/150-153;  
428/328, 330, 331, 320.4-320.8, 411, 488, 537,  
913, 914; 346/210-212, 219, 225, 226

[56] References Cited

U.S. PATENT DOCUMENTS

2,505,471 4/1950 Green ..... 346/225  
2,505,475 4/1950 Green ..... 346/225  
2,505,476 4/1950 Green ..... 346/225  
2,505,477 4/1950 Green ..... 346/225  
2,505,479 4/1950 Green ..... 346/225  
2,505,480 4/1950 Green ..... 346/225  
2,505,483 4/1950 Green ..... 346/225  
2,505,484 4/1950 Green ..... 346/225  
2,505,485 4/1950 Green ..... 346/225  
2,505,486 4/1950 Green ..... 346/225  
2,505,489 4/1950 Green ..... 346/225  
2,618,573 11/1952 Green ..... 346/225  
2,702,765 2/1955 Steinhardt ..... 346/225

2,757,085 7/1956 Pacquin ..... 346/225  
3,223,546 12/1965 Hemstock ..... 346/225  
3,330,722 7/1967 Amano et al. ..... 346/225  
3,565,653 2/1971 Hemstock et al. ..... 346/225  
3,736,285 5/1973 Miller ..... 346/225  
3,980,492 9/1976 Thompson ..... 346/225  
4,022,735 5/1977 Thompson ..... 346/225  
4,038,097 7/1977 Traxler et al. ..... 346/225  
4,109,048 8/1978 Dessauer et al. ..... 346/225  
4,218,504 8/1980 Yamato et al. ..... 346/225

FOREIGN PATENT DOCUMENTS

871604 3/1953 Fed. Rep. of Germany ..... 346/225  
878806 6/1953 Fed. Rep. of Germany ..... 346/225  
1152429 2/1964 Fed. Rep. of Germany ..... 346/225  
2364255 7/1975 Fed. Rep. of Germany ..... 346/225  
3034486 2/1981 Fed. Rep. of Germany ..... 346/225  
38-22819 10/1963 Japan ..... 346/225  
44-2193 1/1969 Japan ..... 346/225  
52-32716 3/1977 Japan ..... 346/225  
628960 9/1949 United Kingdom ..... 346/225  
629165 9/1949 United Kingdom ..... 346/225  
666437 2/1952 United Kingdom ..... 346/225  
710597 6/1954 United Kingdom ..... 346/225  
1271304 4/1972 United Kingdom ..... 346/225  
1307319 2/1973 United Kingdom ..... 346/225  
1392946 5/1975 United Kingdom ..... 346/225  
1445866 8/1976 United Kingdom ..... 346/225  
1451982 10/1976 United Kingdom ..... 346/225  
1467003 3/1977 United Kingdom ..... 346/225  
1497663 1/1978 United Kingdom ..... 346/225

Primary Examiner—Bruce H. Hess

Attorney, Agent, or Firm—Burns, Doane, Swecker & Mathis

[57]

ABSTRACT

A color developer for use in a pressure- or heat-sensitive record material comprises a particulate composite having as components hydrated zirconia and at least one of hydrated silica and hydrated alumina.

4 Claims, No Drawings

## RECORD MATERIAL

This invention relates to record material, and a colour developer for use therein, and to a process for the production of the record material and the colour developer. The record material may be, for example, part of a pressure-sensitive copying system or of a heat-sensitive recording system.

In one known type of pressure-sensitive copying system, usually known as a transfer system, an upper sheet is coated on its lower surface with microcapsules containing a solution of one or more colourless colour formers and a lower sheet is coated on its upper surface with a colour developing co-reactant material. A number of intermediate sheets may also be provided, each of which is coated on its lower surface with microcapsules and on its upper surface with colour developing material. Pressure exerted on the sheets by writing or typing ruptures the microcapsules, thereby releasing the colour former solution on to the colour developing material on the next lower sheet and giving rise to a chemical reaction which develops the colour of the colour former. In a variant of this system, the microcapsules are replaced by a coating in which the colour former solution is present as globules in a continuous matrix of solid material.

In another type of pressure-sensitive copying system, usually known as a self-contained or autogeneous system, microcapsules and colour developing co-reactant material are coated onto the same surface of a sheet, and writing or typing on a sheet placed above the thus-coated sheet causes the microcapsules to rupture and release the colour former, which then reacts with the colour developing material on the sheet to produce a colour.

Heat-sensitive recording systems frequently utilise the same type of reactants as those described above to produce a coloured mark, but rely on heat to convert one or both reactants from a solid state in which no reaction occurs to a liquid state which facilitates the colour-forming reaction, for example by dissolution in a binder which is melted by the heat applied.

The sheet material used in such systems is usually of paper, although in principle there is no limitation on the type of sheet which may be used. When paper is used, the colour developing co-reactant material and/or the microcapsules may be present as a loading within the sheet material instead of as a coating on the sheet material. Such a loading is conveniently introduced into the papermaking stock from which the sheet material is made.

Zirconia, i.e. zirconium dioxide,  $ZrO_2$ , has long been recognised as a material suitable as a co-reactant for developing the colour of colour formers for use in record material, see for example U.S. Pat. Nos. 2505470 and 2777780. However, whilst it is quite effective when in powder form for developing the colour of a solution of a colour former such as crystal violet lactone, it is much less effective when coated on to paper as the active component of a colour developer composition, probably because its reactivity is suppressed by the presence of conventional paper coating binders, for example latex binders. A further problem is that the colour developed initially is very prone to fading.

It has now been found that a composite of hydrated zirconia in major to minor proportion with hydrated silica and/or hydrated alumina will develop a colour

which is of good intensity and has good resistance to fading, particularly when modified by the presence of suitable metal compounds or ions. It should be noted that hydrated zirconia differs from zirconia as referred to above, which is presumed not to be hydrated.

Hydrated silica, various forms of alumina (at least some of which are hydrated) and hydrated silica/hydrated alumina composites have each in themselves been proposed as colour developing materials, see for example U.S. Pat. No. 2828341 in the case of silica, UK Patents Nos. 629165 and 1571325 in the case of alumina, UK Patent No. 1467003 in the case of a hydrated silica/hydrated alumina composite, and UK Patent No. 1271304 in the case of all three of these, the composite in this instance being an aluminate salt precipitated on to hydrated silica. So far as is known however, it had not at the priority date hereof been proposed to utilise a composite of hydrated zirconia with hydrated silica and/or hydrated alumina as a colour developing material.

According to a first aspect of the invention, there is provided record material carrying a colour developer composition which comprises a particulate composite having as components hydrated zirconia and at least one of hydrated silica and hydrated alumina.

According to a second aspect of the invention, there is provided a colour developer for record material, comprising a particulate composite having as components hydrated zirconia and at least one of hydrated silica and hydrated alumina.

According to a third aspect of the invention, there is provided a process for the production of a colour developer for record material, comprising the step of synthesizing in an aqueous medium a particulate composite having as components hydrated zirconia and at least one of hydrated silica and hydrated alumina.

According to a fourth aspect of the invention, there is provided a process for the production of record material, comprising the steps of:

- (a) forming an aqueous dispersion of a particulate composite having as components hydrated zirconia and at least one of hydrated silica and hydrated alumina;
- (b) either:
  - (i) formulating said dispersion into a coating composition and applying the coating composition to a substrate web; or
  - (ii) introducing said dispersion into papermaking stock and forming a paper web which incorporates said composite as a loading; and
- (c) drying the resulting coated or loaded web to produce said record material.

The relative proportions of the components of the composite (i.e. the hydrated zirconia, and either the hydrated silica or the hydrated alumina or both) may vary freely. For example, in the case of a hydrated zirconia/hydrated silica/hydrated alumina composite, these components may be present in approximately equal weight proportion, or any one may predominate, or any two of them may be present in much greater weight proportion than the third. In the case of a hydrated zirconia/hydrated silica composite or a hydrated zirconia/hydrated alumina composite, the hydrated zirconia may be present in major or minor proportion, or the hydrated zirconia and the hydrated silica or hydrated alumina may be present in approximately equal weight proportion.

Preferably however, the proportion of hydrated zirconia is at least 10% by weight of a dry weight basis,

based on the total dry weight of zirconia and silica and/or alumina.

The composite may be synthesized by any of a variety of process routes.

One such route, which in general has been found to be most advantageous is to precipitate at least one of the components on to at least one other of the components. This is thought to result in at least one of the components of the composite (i.e. the later-precipitated component or components) being present in a greater proportion in a surface region of the composite than elsewhere. In the case of a bi-component composite, either of the components may be precipitated in the presence of the other.

Another such route is by precipitation of the components of the composite together from aqueous solution, i.e. from an aqueous solution of a zirconium-containing salt and either an aluminium-containing salt or a silicate salt or both.

A third route is by admixture of previously-formed components of the composite in an aqueous medium, i.e. by admixture of hydrated zirconia and either hydrated silica or hydrated alumina or both. Advantageously, at least one, and preferably all, of the admixed materials are freshly precipitated. At least where hydrated alumina is one of the components of the composite, it may be advantageous to admix the components in an alkaline medium.

In the case of a tri-component composite, any two of the components may be present in aqueous dispersion and the remaining component precipitated in their presence. The two components initially present may have been admixed, or precipitated previously, either together or sequentially. Alternatively, any two of the components may be precipitated from aqueous solution together or sequentially, in the presence of the third.

In a process in which one or more components are precipitated on to another component already in aqueous dispersion, the component already in dispersion may be a material produced in a separate production process, for example a commercially available material, or it may be a material which has been precipitated just previously as an earlier stage in a single process for producing the composite.

Precipitation of hydrated zirconia as part of any of the process routes just described is conveniently carried out by treating a solution of a zirconium salt, for example zirconyl chloride or zirconium sulphate, with an alkaline hydroxide, for example sodium, potassium, lithium or ammonium hydroxide.

Instead of the use of a cationic zirconium salt, hydrated zirconia may be precipitated from a solution of a zirconate, for example ammonium tris-carbonato zirconate, by addition of acid, for example a mineral acid such as sulphuric acid or hydrochloric acid.

Precipitation of hydrated alumina as part of any of the process routes just described is conveniently carried out by treating a solution of a cationic-aluminium salt with an alkaline material such as sodium or potassium hydroxide, although other alkaline materials may be used, for example lithium hydroxide, ammonium hydroxide or calcium hydroxide. It is normally convenient to use aluminium sulphate as the aluminium salt, but other aluminium salts may be used, for example aluminium acetate.

Instead of the use of a cationic aluminium salt, hydrated alumina may be precipitated from a solution of an aluminate, for example sodium or potassium alumi-

nate, by addition of acid, e.g. a mineral acid such as sulphuric or hydrochloric acid.

Precipitation of hydrated silica as part of any of the process routes just described is conveniently carried out by treating a solution of sodium or potassium silicate with an acid, normally one of the common mineral acids such as sulphuric or hydrochloric acid.

The nature of the present colour developing composites has not been fully elucidated, but it is clear from the preparative routes described above that the hydrated zirconia and hydrated silica and/or hydrated alumina elements of the composite are at the least in intimate physical contact and may well be chemically reacted to a greater or lesser degree.

In a preferred embodiment of the present invention, the colour developing composite is modified by the presence of a compound or ions or one or more multivalent metals for example copper, nickel, manganese, cobalt, chromium, zinc, magnesium, titanium, tin, calcium, tungsten, iron, tantalum, molybdenum or niobium. Such modification will hereafter be referred to as "metal modification".

Metal modification may conveniently be brought about by treating the composite, once formed, with a solution of the metal salt, for example the sulphate or chloride. Alternatively, a solution of the metal salt may be introduced into the medium from which the composite or individual components thereof are deposited.

The precise nature of the species formed during metal-modification has not so far been fully elucidated, but one possibility is that a metal oxide or hydroxide is precipitated so as to be present in the composite. An alternative or additional possibility is that ion-exchange occurs so that metal ions are present at ion-exchange sites on the surface of the composite.

Metal modification enables improvements to be obtained in the initial intensity and/or fade resistance of the print obtained from the present colour developing composite with both so-called rapid-developing and so-called slow-developing colour formers, and with colour formers intermediate these categories.

Categorisation of colour formers according to the speed with which their colour may be developed has long been a common practice in the art. 3,3-Bis(4'-dimethylaminophenyl)-6-dimethylaminophthalide (CVL) and similar lactone colour formers are typical of the rapid-developing class, in which colour formation results from cleavage of the lactone ring on contact with an acid co-reactant. 10-Benzoyl-3,7-bis(dime-

thylamino)phenothiazine (more commonly known as benzoyl leuco methylene blue or BLMB) and 10-benzoyl-3,7-bis(diethylamino)phenoxazine (also known as BLASB) are examples of the slow-developing class. It is generally believed that formation of a colour species is

a result of slow hydrolysis of the benzoyl group over a period of up to about two days, followed by aerial oxidation. Spiro-bipyran colour formers, which are widely disclosed in the patent literature, are examples of colour formers in the intermediate category.

The effect achieved by metal modification depends in substantial measure on the particular metal involved and on the particular colour former(s) being used, as will become clear from consideration of the Examples set out hereafter.

The production of the composite by any of the process routes described earlier may take place in the presence of a polymeric rheology modifier such as the sodium salt of carboxymethyl-cellulose (CMC), polyeth-

yleneimine or sodium hexametaphosphate. The presence of such a material modifies the rheological properties of the resulting dispersion of the composite and thus results in a more easily agitatable, pumpable and coatable composition, possibly by having a dispersing or flocculating action. It may be advantageous to form the composite or one or more components thereof in the presence of a particulate material which may function as a carrier or nucleating agent. Suitable particulate materials for this purpose include kaolin, calcium carbonate or other materials commonly used as pigments, fillers or extenders in the paper coating art, since these materials will often need to be included in the coating composition used in the production of a coated record material or in the papermaking stock used in the production of a loaded record material.

A coating composition for use in the production of the present record material will normally also contain a binder (which may be wholly or in part constituted by the CMC optionally used during the preparation of the colour developing material) and/or a filler or extender, which typically is kaolin, calcium carbonate or a synthetic paper coating pigment, for example a urea-formaldehyde resin pigment. The filler or extender may be wholly or in part constituted by the particulate material which may be used during the preparation of the composite. In the case of a loaded record material, a filler or extender may also be present, and again this may be wholly or in part constituted by the particulate material which may be used during the preparation of the composite.

The pH of the coating composition influences the subsequent colour developing performance of the composition, and also its viscosity, which is significant in terms of the ease with which the composition may be coated on to paper or another substrate. The preferred pH for the coating composition is within the range 5 to 9.5, and is preferably around 7.0. Sodium hydroxide is conveniently used for pH adjustment, but other alkaline materials may be used, for example potassium hydroxide, lithium hydroxide, calcium hydroxide, ammonium hydroxide, sodium silicate, or potassium silicate.

The aqueous dispersion which is formulated into the coating composition or introduced into the papermaking stock may be the dispersion obtained as a result of synthesis of the composite in the aqueous medium. Alternatively, the composite may be separated after its synthesis, e.g. by filtering off, and then washed to remove soluble salts before being re-dispersed in a further aqueous medium to form the dispersion for formulation into the coating composition or introduction into the paper-making stock.

The present composite may be used as the only colour developing material in a colour developing composition, or it may be used together with other colour developing materials, e.g. an acid-washed dioctahedral montmorillonite clay, a phenolic resin, or a salicylic acid derivative.

It is usually desirable to treat the composite in order to break up any aggregates which have formed, for example by ball-milling. This treatment may be carried out either before or after the optional addition of fillers and/or additional colour developing materials.

In the case of a coated record material, the record material may form part of a transfer or self-contained pressure-sensitive copying system or of a heat-sensitive recording system as described previously. In the case of a loaded record material, the record material may be

used in the same manner as the coated record material just described, or the record material may also carry microencapsulated colour former solution as a loading, so as to be a self-contained record material.

The invention will now be illustrated by the following Examples (in which all percentages quoted are by weight):

#### EXAMPLE 1

10 This illustrates the production of a series of hydrated silica/hydrated zirconia/hydrated alumina composites with different relative proportions of hydrated silica, hydrated zirconia and hydrated alumina by a process in which the hydrated zirconia, hydrated silica and hydrated alumina are precipitated together from a common aqueous solution.

Z g of dry zirconyl chloride,  $ZrOCl_2 \cdot 8H_2O$  were dissolved in A g of a 40% w/w solution of aluminium sulphate,  $Al_2(SO_4)_3 \cdot 16H_2O$ . S g of a solution of sodium silicate (Pyramid 120 supplied by Joseph Crosfield & Sons Ltd., but diluted from its as-supplied solids content of 48% to 24% solids content) were then added slowly, whilst maintaining the pH of the resulting mixture below 4.0. When all the sodium silicate solution has been added the pH of the mixture was adjusted to 7.0 using sodium hydroxide solution. The foregoing procedure resulted in formation of a slurry of a hydrated silica/hydrated zirconia/hydrated alumina composite. The slurry was ball milled by passage through a continuous laboratory ball mill, after which it was filtered. The material collected was washed with de-ionized water so as to remove substantially all water-soluble salts. The washed material was then re-dispersed in de-ionized water and 8.82 g of 50% solids content styrene-butadiene latex binder (that supplied by Dow as Dow 675 latex) were added, giving a 15% latex content on a dry weight basis in each case. Sufficient water was added to lower the viscosity of the mixture to a level suitable for coating using a laboratory Meyer Bar coater. The mixture was then coated on to paper at a nominal dry coatweight of  $8 \text{ gm}^{-2}$ , and the coated sheet was dried at  $110^\circ \text{C}$ . and calendered. The finished sheet was then subjected to calender intensity and fade resistance tests to assess its performance as a colour developing material.

The values of Z, A and S are set out below:

|           | Z (g) | A (g) | S (g) |
|-----------|-------|-------|-------|
| Run No. 1 | 43.2  | 254.8 | 103.1 |
| Run No. 2 | 26.2  | 154.4 | 187.5 |
| Run No. 3 | 26.2  | 463.2 | 62.5  |
| Run No. 4 | 78.5  | 154.4 | 62.5  |

The resulting silica, zirconia and alumina contents of the composite on a dry weight basis, based on the total dry weight of silica, zirconia and alumina are set out below:

|           | % $SiO_2$ | % $ZrO_2$ | % $Al_2O_3$ |
|-----------|-----------|-----------|-------------|
| Run No. 1 | 33.3      | 33.3      | 33.3        |
| Run No. 2 | 60        | 20        | 20          |
| Run No. 3 | 20        | 20        | 60          |
| Run No. 4 | 20        | 60        | 20          |

The calender intensity test involved superimposing a strip of paper coated with encapsulated colour former

solution on a strip of the coated paper under test, passing the superimposed strips through a laboratory calender to rupture the capsules and thereby produce a colour on the test strip, measuring the reflectance of the coloured strip (I) and expressing the results ( $I/I_0$ ) as a percentage of the reflectance of an unused control strip ( $I_0$ ). Thus the lower the calender intensity value ( $I/I_0$ ) the more intense the developed colour. The calender intensity tests were done with a paper ("Paper A") which employed a commercially used colour former blend containing, inter alia, CVL as a rapid-developing colour former and BLASB as a slow-developing colour former.

The reflectance measurements were done both two minutes after calendering and forty-eight hours after calendering, the sample being kept in the dark in the interim. The colour developed after two minutes is primarily due to the rapid-developing colour formers, whereas the colour after forty-eight hours derives also from the slow-developing colour formers (fading of the colour from the rapid-developing colour formers also influences the intensity achieved).

The fading test involved positioning the developed strips (after forty-eight hours development) in a cabinet in which were an array of daylight fluorescent strip-plamps. This is thought to simulate, in accelerated form, the fading which a print might undergo under normal conditions of use. After exposure for the desired time, measurements were made as described with reference to the calender intensity test, and the results were expressed in the same way.

The calender intensity and fade resistance results were as follows:

| Test<br>Conditions | Run No. |      |      |      |
|--------------------|---------|------|------|------|
|                    | 1       | 2    | 3    | 4    |
| 2 min development  | 34.1    | 41.0 | 35.1 | 33.9 |
| 48 hr development  | 30.3    | 36.9 | 28.1 | 30.7 |
| 15 hr fade         | 51.0    | 58.2 | 49.3 | 50.5 |
| Intensity Decline* | 20.7    | 21.3 | 21.2 | 19.8 |

\*The "intensity decline" in this and subsequent Examples is a measure of the extent of fading from the intensity value reached after 48 hours dark development.

## EXAMPLE 2

This illustrates metal modification of a hydrated silica/hydrated zirconia/hydrated alumina composite, produced by a process generally as described in Example 1, the particular modifying metal in this instance being copper. The procedure was as described in Example 1 (Run No. 1), except firstly that after adjustment of the pH to 7.0, 2.4 g of copper sulphate,  $\text{CuSO}_4 \cdot 5\text{H}_2\text{O}$  were added and the slurry was stirred for about 10 minutes, and secondly that 8.96 g of latex were used.

The resulting copper modification level was 1.5%, calculated as cupric oxide on a dry weight basis, based on the total dry weight of silica, zirconia, alumina and cupric oxide.

The calender intensity and fade resistance values were as follows:

|                    |      |
|--------------------|------|
| 2 min. development | 36.6 |
| 48 hr. development | 32.0 |
| 15 hr. fade        | 48.3 |
| Intensity decline  | 16.3 |

It will be seen that copper modification resulted in a slightly worse initial intensity but a significantly im-

proved fade resistance (a fall of 16.3 points rather than 20.7 points).

## EXAMPLE 3

This illustrates the production of a series of hydrated silica/hydrated zirconia/hydrated alumina composites with different relative proportions of hydrated silica, hydrated zirconia and hydrated alumina by a process in which freshly prepared hydrated silica, freshly prepared hydrated zirconia and freshly prepared hydrated alumina are admixed.

A master batch of hydrated silica slurry was prepared by neutralizing sodium silicate solution to pH 7.0 with 40% w/w sulphuric acid. The resulting hydrated silica precipitate was filtered off and washed with de-ionized water to remove water-soluble salts. The washed precipitate was then re-dispersed in de-ionized water and the resulting slurry was passed through a continuous laboratory ball-mill, after which it was filtered. The collected material was washed to remove any remaining water soluble salts, and then re-dispersed in de-ionized water. The solids content of the resulting slurry was measured and found to be 16.5%.

A master batch of hydrated alumina slurry was prepared by neutralizing a 40% w/w solution of aluminium sulphate,  $\text{Al}_2(\text{SO}_4)_3 \cdot 16\text{H}_2\text{O}$  to pH 7.0 by slow addition of 40% w/w sodium hydroxide solution with vigorous stirring. The resulting hydrated alumina precipitate was filtered off and washed twice with de-ionized water to remove water-soluble salts. The washed precipitate was then re-dispersed in de-ionized water and the resulting slurry was passed through a continuous laboratory ball-mill, after which it was filtered. The collected material was re-washed, re-dispersed and filtered off again, before final re-dispersion in de-ionized water. The solids content of the slurry was measured and found to be 12.5%.

A master batch of hydrated zirconia slurry was prepared by neutralizing a solution of zirconyl chloride,  $\text{ZrOCl}_2 \cdot 8\text{H}_2\text{O}$  to pH 7.0 with 40% w/w sodium hydroxide solution. The resulting hydrated zirconia precipitate was filtered off and washed with de-ionized water to remove water-soluble salts. The washed precipitate was then re-dispersed in de-ionized water and the resulting slurry was passed through a continuous laboratory ball-mill, after which it was filtered. The collected material was then re-dispersed in de-ionized water. The solids content of the resulting slurry was measured and found to be 19.1%.

S g of the hydrated silica slurry, A g of the hydrated alumina slurry and Z g of the hydrated zirconia slurry were then mixed and 7.5 g of latex (Dow 675) were added, giving a latex level of 15% on a dry weight basis in each case. The experimental and testing procedures from this point on were as described in Example 1.

The values of Z, A and S are set out below:

|           | Z (g) | A (g) | S (g) |
|-----------|-------|-------|-------|
| Run No. 1 | 43.2  | 66.0  | 50.0  |
| Run No. 2 | 78.6  | 40.0  | 30.3  |
| Run No. 3 | 26.2  | 40.0  | 90.9  |
| Run No. 4 | 26.2  | 120.0 | 30.3  |

The resulting silica, zirconia and alumina contents of the composite on a dry weight basis, based on the total dry weight of silica, zirconia and alumina are set out below:

|           | % SiO <sub>2</sub> | % ZrO <sub>2</sub> | % Al <sub>2</sub> O <sub>3</sub> |
|-----------|--------------------|--------------------|----------------------------------|
| Run No. 1 | 33.3               | 33.3               | 33.3                             |
| Run No. 2 | 20                 | 60                 | 20                               |
| Run No. 3 | 60                 | 20                 | 20                               |
| Run No. 4 | 20                 | 20                 | 60                               |

The calender intensity and fade resistance results obtained were as follows:

| Test<br>Conditions | Run No. |      |      |      |
|--------------------|---------|------|------|------|
|                    | 1       | 2    | 3    | 4    |
| 2 min. development | 43.9    | 51.0 | 45.9 | 52.6 |
| 48 hr. development | 42.0    | 46.5 | 43.2 | 49.1 |
| 15 hr. fade        | 59.4    | 66.9 | 62.3 | 65.4 |
| Intensity decline  | 17.4    | 20.4 | 19.1 | 16.3 |

#### EXAMPLE 4

This illustrates metal modification of a hydrated silica/hydrated zirconia/hydrated alumina composite produced by a process generally as described in Example 3, the particular modifying metal in this instance being copper. The procedure was as described in Example 3 (Run No. 4), except that before the latex addition, 1.08 g of copper sulphate, CuSO<sub>4</sub>.5H<sub>2</sub>O were added and the slurry was stirred for 10 minutes.

The resulting copper modification level was 1.5% calculated on the same basis as in Example 2.

The calender intensity and fade resistance values were as follows:

|                    |      |
|--------------------|------|
| 2 min development  | 51.9 |
| 48 hr. development | 48.8 |
| 15 hr. fade        | 61.8 |
| Intensity decline  | 13.0 |

It will be seen that copper modification resulted in improved fade resistance.

#### EXAMPLE 5

This illustrates the production of a hydrated zirconia/hydrated alumina composite in which hydrated zirconia predominates by a process in which hydrated zirconia and hydrated alumina are precipitated sequentially.

2.4 g of CMC (FF5 supplied by Finnfix) were dissolved in 210 g of de-ionized water over a period of 15 minutes with stirring. 90 g of zirconyl chloride, ZrOCl<sub>2</sub>.8H<sub>2</sub>O were then added, giving an acidic solution, and 40% w/w sodium hydroxide solution was added slowly with stirring to restore the pH to 7.0, with resultant precipitation of hydrated zirconia. Approximately 60 g of the sodium hydroxide solution was required for this purpose. The mixture was left stirring for an hour, after which it was ball-milled overnight. The mixture was then split into five portions, four of 50 g and one of 60 g. X g of 40% w/w solution of aluminium sulphate, Al<sub>2</sub>(SO<sub>4</sub>)<sub>3</sub>.16H<sub>2</sub>O were then added to each 50 g portion, and the pH of each mixture was readjusted to 7 by the addition of further sodium hydroxide solution. This resulted in precipitation of hydrated alumina onto the hydrated zirconia to form a hydrated zirconia/hydrated alumina composite. Each mixture was left stirring for an hour, after which 2.8 g of kaolin (Dinkie A supplied by English China Clays) were added (3.3 g in the case of the slurry to which aluminium sulphate

solution had not been added). After stirring each mixture for a further 30 minutes, 2.8 g of latex (Dow 675) were added (3.3 g in the case of the slurry to which aluminium sulphate had not been added). After further stirring, the mixtures were coated onto respective sheets of paper at a nominal dry coatweight of 8 gm<sup>-2</sup> using a laboratory Meyer bar coater. The coated sheets were then dried and calendered and subjected to calender intensity and fade resistance tests to assess their performance as colour developing materials.

The values of X and the resulting alumina content of the hydrated zirconia/hydrated alumina composites, on a dried weight basis, based on the total dry weight of zirconia and alumina were as follows:

| Mix No. | X (g) | % Al <sub>2</sub> O <sub>3</sub> |
|---------|-------|----------------------------------|
| 1       | 0     | 0                                |
| 2       | 8.1   | 10                               |
| 3       | 8.1   | 10                               |
| 4       | 18.3  | 20                               |
| 5       | 48.8  | 40                               |

The calender intensity test was generally as described in Example 1, except that testing was carried out with three different microcapsule coated papers. One of these was Paper A as described in Example 1. Another ("Paper B") employed an experimental colour former blend including CVL, a slow-developing blue colour former and an intermediate-developing colour former which was a spiro-bipyran derivative. The third paper ("Paper C") employed CVL as the sole colour former.

The results of the calender intensity and fade resistance tests were as follows:

| Test<br>Conditions  | Paper A |               |               |      |      |
|---------------------|---------|---------------|---------------|------|------|
|                     | 0       | 10<br>(Mix 2) | 10<br>(Mix 3) | 20   | 40   |
| 2 min. development  | 63.7    | 45.4          | 45.1          | 45.3 | 47.0 |
| 48 hour development | 44.7    | 37.8          | 37.4          | 37.2 | 37.7 |
| 1 hour fade         | 44.0    | 37.9          | 37.7          | 36.7 | 36.1 |
| 15 hour fade        | 63.5    | 56.3          | 54.3          | 50.4 | 52.2 |
| Intensity decline   | 18.8    | 18.5          | 16.9          | 13.2 | 14.5 |

| Test<br>Conditions  | Paper B |               |               |      |      |
|---------------------|---------|---------------|---------------|------|------|
|                     | 0       | 10<br>(Mix 2) | 10<br>(Mix 3) | 20   | 40   |
| 2 min. development  | 68.5    | 50.7          | 50.8          | 45.3 | 52.0 |
| 48 hour development | 52.8    | 45.0          | 45.2          | 37.2 | 45.4 |
| 1 hour fade         | 48.6    | 43.3          | 43.4          | 36.9 | 42.3 |
| 15 hour fade        | 60.1    | 55.7          | 57.2          | 50.9 | 59.1 |
| Intensity decline   | 7.3     | 10.7          | 12.0          | 13.7 | 13.7 |

| Test<br>Conditions  | Paper C |               |               |      |      |
|---------------------|---------|---------------|---------------|------|------|
|                     | 0       | 10<br>(Mix 2) | 10<br>(Mix 3) | 20   | 40   |
| 2 min. development  | 71.5    | 60.1          | 59.5          | 59.6 | 62.9 |
| 48 hour development | 62.4    | 57.1          | 57.3          | 56.6 | 58.4 |
| 1 hour fade         | 66.1    | 59.1          | 59.2          | 58.0 | 66.4 |
| 15 hour fade        | 89.6    | 80.2          | 79.8          | 76.9 | 77.7 |
| Intensity decline   | 27.2    | 23.1          | 22.5          | 20.3 | 19.3 |

It will be seen that the inclusion of hydrated alumina improved the initial intensity and/or fade resistance obtained in each case.

## EXAMPLE 6

This illustrates metal modification of a hydrated zirconia/hydrated alumina composite in which hydrated zirconia predominates and which is produced by a process generally as described in Example 5, using a variety of modifying metals.

1.2 g of CMC were dissolved in 105 g of de-ionized water over a period of 15 minutes with stirring. 45 g of zirconyl chloride,  $ZrOCl_2 \cdot 8H_2O$  were then added, giving an acidic solution, and 40% w/w sodium hydroxide solution was added slowly with stirring to restore the pH to 7.0, with resultant precipitation of hydrated zirconia. About 30 g of the sodium hydroxide solution was required for this purpose. The mixture was left stirring for an hour, after which 29.5 g of 40% w/w solution of aluminium sulphate  $Al_2(SO_4)_3 \cdot 16H_2O$  were added and the pH was readjusted to 7 by the addition of further sodium hydroxide solution. This resulted in precipitation of hydrated alumina. The mixture was left stirring for an hour, after which X g of a metal compound M were added. The pH was then re-adjusted to 7.0 by the addition of further sodium hydroxide solution, and stirring was continued for a further hour. Kaolin and latex were successively added (10 g in each case) following the procedure described in Example 5 and the compositions were coated onto paper and tested, as described in Example 5. A control procedure with no modifying metal compound was also carried out.

The value of X and the nature of M were as follows:

| X (g) | M                                                         |
|-------|-----------------------------------------------------------|
| 4.5   | Copper sulphate $CuSO_4 \cdot 5H_2O$                      |
| 0.8   | Phosphomolybdic acid $12MoO_3 \cdot H_3PO_4 \cdot 24H_2O$ |
| 1.8   | Nickel chloride $NiCl_2 \cdot 6H_2O$                      |
| 0.6   | Niobium pentoxide $Nb_2O_5$                               |
| 1.2   | Stannic chloride $SnCl_4 \cdot 5H_2O$                     |
| 0.6   | Titanium dioxide $TiO_2$                                  |
| 0.7   | Phosphotungstic acid $H_3PO_4 \cdot 12WO_3 \cdot xH_2O$   |
| 1.0   | Zinc chloride $ZnCl_2$                                    |
| 1.6   | Ferrous chloride $FeCl_2 \cdot 4H_2O$                     |

The results of calender intensity and fade resistance tests were as follows:

| Test                | Modifying metal |      |      |      |      |
|---------------------|-----------------|------|------|------|------|
|                     | None            | Cu   | Mo   | Ni   | Nb   |
| 2 min. development  | 48.0            | 46.3 | 46.9 | 48.8 | 46.1 |
| 48 hour development | 38.0            | 39.4 | 41.0 | 40.6 | 37.7 |
| 1 hour fade         | 41.0            | 40.1 | 42.6 | 42.3 | 40.5 |
| 3 hour fade         | 51.3            | 42.8 | 48.4 | 47.2 | 45.7 |
| 5 hour fade         | 55.0            | 45.9 | 55.3 | 51.6 | 53.4 |
| 10 hour fade        | 63.5            | 49.7 | 63.4 | 59.2 | 61.6 |
| 15 hour fade        | 73.0            | 60.0 | 73.0 | 69.1 | 71.3 |
| Intensity decline   | 35.0            | 20.6 | 32.0 | 28.5 | 33.6 |

| Test                | Modifying metal |      |      |      |      |
|---------------------|-----------------|------|------|------|------|
|                     | Sn              | Ti   | W    | Zn   | Fe   |
| 2 min. development  | 46.2            | 48.2 | 47.7 | 44.0 | 47.6 |
| 48 hour development | 40.8            | 40.9 | 39.8 | 37.4 | 38.5 |

-continued

| Test              | Modifying metal |      |      |      |      |
|-------------------|-----------------|------|------|------|------|
|                   | Sn              | Ti   | W    | Zn   | Fe   |
| 1 hour fade       | 40.6            | 41.5 | 41.4 | 40.8 | 42.2 |
| 3 hour fade       | 45.0            | 46.1 | 47.4 | 47.2 | 56.7 |
| 5 hour fade       | 50.0            | 52.7 | 53.7 | —    | —    |
| 10 hour fade      | 60.2            | 63.8 | 64.8 | —    | —    |
| 15 hour fade      | 67.5            | 69.8 | 70.7 | —    | —    |
| Intensity decline | 26.7            | 28.9 | 30.9 | 9.8  | 18.2 |

| Test                | Paper B Modifying metal |      |      |      |      |
|---------------------|-------------------------|------|------|------|------|
|                     | None                    | Cu   | Mo   | Ni   | Nb   |
| 2 min. development  | 54.6                    | 51.0 | 56.6 | 58.0 | 55.5 |
| 48 hour development | 45.5                    | 45.7 | 49.8 | 49.0 | 46.7 |
| 1 hour fade         | 46.6                    | 46.3 | 48.2 | 47.7 | 45.8 |
| 3 hour fade         | 55.6                    | 48.4 | 51.9 | 50.7 | 49.6 |
| 5 hour fade         | —                       | 50.3 | 56.6 | 54.1 | 53.9 |
| 10 hour fade        | —                       | 54.1 | 62.5 | 59.3 | 59.6 |
| 15 hour fade        | —                       | 60.3 | 72.6 | 66.3 | 66.1 |
| Intensity decline   | 10.1                    | 14.6 | 22.8 | 17.3 | 19.4 |

| Test                | Modifying metal |      |      |      |      |
|---------------------|-----------------|------|------|------|------|
|                     | Su              | Ti   | W    | Zn   | Fe   |
| 2 min. development  | 55.1            | 55.7 | 56.9 | 50.7 | 53.5 |
| 48 hour development | 48.9            | 48.3 | 48.4 | 44.4 | 45.5 |
| 1 hour fade         | 47.2            | 47.7 | 47.9 | 44.9 | 45.9 |
| 3 hour fade         | 50.6            | 52.1 | 50.6 | 50.0 | 55.5 |
| 5 hour fade         | 55.3            | 57.4 | 56.7 | —    | —    |
| 10 hour fade        | 62.7            | 64.0 | 64.2 | —    | —    |
| 15 hour fade        | 66.0            | 68.0 | 67.9 | —    | —    |
| Intensity decline   | 17.1            | 19.7 | 19.5 | 5.6  | 10.0 |

| Test                | Paper C Modifying metal |      |      |      |      |
|---------------------|-------------------------|------|------|------|------|
|                     | None                    | Cu   | Mo   | Ni   | Nb   |
| 2 min. development  | 62.8                    | 62.5 | 63.2 | 62.8 | 61.8 |
| 48 hour development | 58.7                    | 59.4 | 58.8 | 59.3 | 58.4 |
| 1 hour fade         | 63.8                    | 60.0 | 64.6 | 62.0 | 63.7 |
| 3 hour fade         | 76.9                    | 63.4 | 72.5 | 66.6 | 70.4 |
| 5 hour fade         | 79.2                    | 65.7 | 77.9 | 70.8 | 75.7 |
| 10 hour fade        | 88.1                    | 71.8 | 86.1 | 77.4 | 84.7 |
| 15 hour fade        | 95.0                    | 81.7 | 94.3 | 86.5 | 93.5 |
| Intensity decline   | 36.3                    | 22.3 | 35.5 | 27.2 | 35.1 |

| Test                | Modifying metal |      |      |      |      |
|---------------------|-----------------|------|------|------|------|
|                     | Sn              | Ti   | W    | Zn   | Fe   |
| 2 min. development  | 63.3            | 63.7 | 62.6 | 60.8 | 62.5 |
| 48 hour development | 59.4            | 59.4 | 58.5 | 56.8 | 58.1 |
| 1 hour fade         | 62.8            | —    | 64.7 | 62.5 | 63.0 |
| 3 hour fade         | 66.0            | —    | 70.5 | 72.8 | 77.7 |
| 5 hour fade         | 71.3            | —    | 76.1 | —    | 80.0 |
| 10 hour fade        | 80.9            | —    | 89.4 | —    | 87.5 |
| 15 hour fade        | 87.3            | 82.6 | 93.1 | —    | 93.8 |
| Intensity decline   | 27.9            | 23.2 | 34.6 | 16.0 | 35.7 |

It will be seen that whilst some metals are much more effective as modifiers than others, all of them gave improved performance in at least some respects.

#### EXAMPLE 7

This illustrates the production of a hydrated zirconia/hydrated silica composite in which hydrated silica predominates by a process in which freshly precipitated hydrated zirconia is admixed with hydrated silica.

50 g of zirconyl chloride,  $ZrOCl_2 \cdot 8H_2O$  were dissolved in 100 g de-ionized water. This solution was neutralized to pH 7.0 by the addition of aqueous ammonia, and the resulting hydrated zirconia precipitate was filtered off and washed with de-ionized water to remove soluble salts. This preparative procedure was carried out six times in all to produce six batches of hydrated zirconia. The zirconia content on a dry weight basis was measured and found to be 19.1%.

A series of parallel experiments was then carried out 20 in which X g of one batch of the hydrated zirconia were dispersed in 50 g de-ionized water and Y g of hydrated silica were added.

The mixture was stirred for an hour and the pH was readjusted to 7.0 (if necessary). Z g of a 50% solids content styrene butadiene latex binder (Dow 675) were added with stirring. The experimental and test procedures from this point on were as described in Example 1. Control experiments with no hydrated silica addition and with no hydrated zirconia present were also carried out for comparison purposes.

The values of X, Y and Z and the silica content of the composite on a dried weight basis, based on the total dry weight of silica and zirconia, are set out below:

| X (g) | Y (g) | Z (g) | % $SiO_2$ |
|-------|-------|-------|-----------|
| 100   | 0     | 8     | 0         |
| 110   | 11.2  | 8.6   | 10        |
| 105   | 25.3  | 9.4   | 20        |
| 100   | 43.4  | 10.0  | 30        |
| 105   | 67.3  | 11.2  | 40        |
| 105   | 101.1 | 13.2  | 50        |

The calender intensity and fade resistance results were as follows:

| Test Conditions     | % $SiO_2$ |      |      |      |      |      |      |
|---------------------|-----------|------|------|------|------|------|------|
|                     | 0         | 10   | 20   | 30   | 40   | 50   | 100  |
| 2 min. development  | 61.0      | 48.8 | 48.5 | 48.6 | 46.8 | 46.4 | 55.0 |
| 48 hour development | 54.6      | 40.9 | 41.9 | 42.1 | 40.5 | 40.9 | 54.8 |
| 15 hour fade        | 77.1      | 69.3 | 70.6 | 72.3 | 73.5 | 75.4 | 81.5 |
| Intensity decline   | 22.5      | 28.4 | 28.7 | 30.2 | 33.0 | 34.5 | 26.7 |

It will be seen that the inclusion of hydrated silica resulted in enhanced initial intensity, compared with hydrated zirconia alone. It will also be noted that the colour developing performance of the composite was superior to that of hydrated silica alone.

#### EXAMPLE 8

This illustrates metal modification of a hydrated zirconia/hydrated silica composite produced by a process generally as described in Example 7, using a variety of modifying metals.

Batches of hydrated zirconia/hydrated silica composite containing 10% silica on a dried weight basis, based on the total dry weight of zirconia and silica,

were prepared as in Example 7, except that X g of a metal compound M were added prior to the final pH adjustment and latex addition. A control batch with no metal compound addition was also prepared for comparison purposes. Coated sheets were then prepared and tested as described in Example 1.

The values of X g and the nature of M were as follows:

| 10   | X (g)              | M                    |
|------|--------------------|----------------------|
| 0.81 | Ferrous sulphate   | $FeSO_4 \cdot 7H_2O$ |
| 0.82 | Cobalt sulphate    | $CoSO_4 \cdot 7H_2O$ |
| 0.81 | Nickel sulphate    | $NiSO_4 \cdot 7H_2O$ |
| 0.73 | Copper sulphate    | $CuSO_4 \cdot 5H_2O$ |
| 0.39 | Calcium sulphate   | $CaSO_4$ (anhydrous) |
| 0.71 | Magnesium sulphate | $MgSO_4 \cdot 7H_2O$ |
| 0.83 | Zinc sulphate      | $ZnSO_4 \cdot 7H_2O$ |

The calender intensity and fade resistance results obtained were as follows:

| Test Conditions     | Metal |      |      |      |      |      |      |      |
|---------------------|-------|------|------|------|------|------|------|------|
|                     | —     | Fe   | Co   | Ni   | Cu   | Ca   | Mg   | Zn   |
| 2 min. development  | 48.8  | 44.3 | 44.8 | 48.2 | 39.5 | 46.7 | 43.9 | 44.3 |
| 48 hour development | 40.9  | 39.1 | 38.6 | 40.1 | 33.1 | 39.3 | 38.5 | 39.1 |
| 15 hour fade        | 69.3  | 63.3 | 55.0 | 60.8 | 47.5 | 64.4 | 69.2 | 65.3 |
| Intensity decline   | 28.4  | 24.2 | 16.4 | 20.7 | 14.4 | 25.1 | 30.7 | 26.2 |

It will be seen that metal modification enhanced initial intensity and/or fade resistance.

#### EXAMPLE 9

This illustrates the production of a hydrated zirconia/hydrated silica composite in which hydrated zirconia predominates by a process in which hydrated zirconia is precipitated on to freshly-precipitated hydrated silica.

A master batch of hydrated silica slurry was first prepared by neutralizing sodium silicate solution (Pyramid 120 supplied by Joseph Crosfield & Sons Ltd. at 48% solids content) to pH 7.0 with 40% w/w sulphuric acid. The resulting hydrated silica precipitate was filtered off and washed three times with de-ionized water so as to remove substantially all water-soluble salts. The washed precipitate was then re-dispersed in de-ionized water. The silica content on a dry weight basis was checked and found to be approximately 20%.

Two parallel experiments were then carried out in which X g of zirconyl chloride,  $ZrOCl_2 \cdot 8H_2O$  were added in each case to an amount of the above-prepared hydrated slurry equivalent to Y g silica on a dry weight basis. The pH was then adjusted to 7.0 with 10N sodium hydroxide solution, with resultant formation of a hydrated zirconia/hydrated silica composite. Z g of 50% solids content styrene-butadiene latex binder (Dow 675) were added. The value of Z g was selected to give an equivalent binder level in each case (15% on a dry weight basis). The experimental and test procedures from this point on were as described in Example 1.

The values of X, Y and Z and the zirconia content of the composite on a dry weight basis, based on the total dry weight of zirconia and silica, are set out below:

| X    | Y    | Z   | % ZrO <sub>2</sub> |
|------|------|-----|--------------------|
| 0    | 25.0 | 7.5 | 0                  |
| 26.9 | 7.5  | 5.4 | 57.7               |
| 38.6 | 6.3  | 5.7 | 67.2               |

The calendar intensity and fade resistance results were as follows:

| Test                | % ZrO <sub>2</sub> |      |      |
|---------------------|--------------------|------|------|
| Conditions          | 57.7               | 67.2 | 0    |
| 2 min. development  | 50.1               | 54.8 | 47.1 |
| 48 hour development | 44.8               | 44.9 | 36.6 |
| 15 hour fade        | 70.3               | 70.7 | 76.4 |
| Intensity decline   | 25.5               | 25.8 | 39.8 |

It will be seen that the composite gave much improved fade resistance compared with hydrated silica alone.

### EXAMPLE 10

This illustrates the production of a series of hydrated zirconia/hydrated alumina composites in which hydrated alumina predominates (or, in one case, in which the hydrated zirconia and hydrated alumina are present in equal weight proportions) by a process in which hydrated zirconia is precipitated on to freshly-precipitated hydrated alumina.

A master batch of hydrated alumina slurry was first prepared by neutralizing a 40% w/w solution of aluminium sulphate,  $\text{Al}_2(\text{SO}_4)_3 \cdot 16\text{H}_2\text{O}$  to pH 7.0 by the slow addition with vigorous stirring of 10N sodium hydroxide solution. The resulting hydrated alumina precipitate was filtered off and washed three times with de-ionized water so as to remove substantially all water-soluble salts. The washed precipitate was then redispersed in de-ionized water, and the resulting slurry was ball-milled to reduce the median particle size from an initial value of approximately 8  $\mu\text{m}$  to approximately 4  $\mu\text{m}$  (as measured by a Coulter Counter). The alumina content on a dry weight basis was then checked and found to be approximately 22.8%.

A series of parallel experiments was then carried out in which X g of zirconyl chloride,  $ZrOCl_2 \cdot 8H_2O$  were added in each case to 100 g of the above-prepared hydrated alumina slurry (equivalent to 22.8 g alumina on a dry weight basis). The pH was then adjusted to 7.0 by the addition of 10N sodium hydroxide solution, with resultant formation of a hydrated alumina/hydrated zirconia composite. This was filtered off and washed with de-ionized water to remove soluble salts. The washed material was then re-dispersed in de-ionized water and Y g of latex binder (Dow 675) were added. The value of Y was selected to give an equivalent binder level in each case. The experimental and test procedures from this point on were as described in Example 1. A control experiment with no zirconyl chloride addition was also carried out for comparison purposes.

The values of X and Y and the zirconia content of the composite on a dry weight basis, based on the total dry weight of zirconia and alumina, are set out below:

-continued

| X (g) | Y (g) | % ZrO <sub>2</sub> |
|-------|-------|--------------------|
| 6.61  | 8.94  | 10                 |
| 14.82 | 10.06 | 20                 |
| 25.54 | 11.50 | 30                 |
| 39.67 | 13.41 | 40                 |
| 59.51 | 16.10 | 50                 |

10 The calendar intensity and fade resistance results  
11 were as follows:

| Test                 | % ZrO <sub>2</sub> |      |      |      |      |
|----------------------|--------------------|------|------|------|------|
| Conditions           | 0                  | 10   | 20   | 30   | 40   |
| 2 min. development   | 43.3               | 39.3 | 40.7 | 40.2 | 39.0 |
| 48 hours development | 36.3               | 32.9 | 33.8 | 33.7 | 33.8 |
| 15 hours fade        | 65.3               | 50.1 | 50.4 | 52.0 | 56.5 |
| Intensity decline    | 29.0               | 17.2 | 16.6 | 18.3 | 22.7 |

20 It will be seen that the presence of hydrated zirconia improved the initial intensity and fade resistance in all cases, compared with hydrated alumina alone.

**EXAMPLE 11**

25 This illustrates metal modification of a hydrated zirconia/hydrated alumina composite produced by a process generally as described in Example 10, using a variety of modifying metals.

30 A master batch of hydrated zirconia/hydrated alumina composite having a 20% zirconia content on a dried weight basis, based on the total dry weight of zirconia and alumina, was made up by the method described in Example 10, except that larger quantities were used. The composite was found to have a solids content of 18.3%.

A series of parallel experiments was then carried out in which  $X$  g of a metal compound  $M$  were added in each case to 150 g of the composite. The resulting slurry was filtered, and the filtered off material was washed 40 with de-ionized water to remove soluble salts. The washed material was then redispersed in de-ionized water and 9.69 g of latex binder (Dow 675) were added. The experimental and test procedures from this point on were as described in Example 1. A control experiment 45 with no metal-modification was also carried out for comparison purposes.

The value of X and the nature of M were as set out below (it should be noted that the value of X was chosen to give a 1.5% metal modification level on a dried weight basis, calculated as the weight of metal oxide in relation to the total weight of zirconia, alumina and metal oxide).

| 55 | X (g) | M                  |
|----|-------|--------------------|
|    | 1.63  | Ferrous sulphate   |
|    | 1.63  | Cobalt sulphate    |
|    | 1.63  | Nickel sulphate    |
|    | 1.31  | Copper sulphate    |
|    | 2.57  | Magnesium sulphate |
| 60 | 1.63  | Calcium chloride   |
|    | 1.49  | Zinc sulphate      |

The results obtained were as follows:

| Test<br>Conditions | Metal |      |      |      |      |      |      |      |
|--------------------|-------|------|------|------|------|------|------|------|
|                    | —     | Fe   | Co   | Ni   | Cu   | Mg   | Ca   | Zn   |
| 2 min.             | 35.7  | 36.0 | 36.5 | 35.4 | 34.9 | 33.5 | 33.3 | 33.6 |

-continued

| Test<br>Conditions   | Metal |      |      |      |      |      |      |      |
|----------------------|-------|------|------|------|------|------|------|------|
|                      | —     | Fe   | Co   | Ni   | Cu   | Mg   | Ca   | Zn   |
| development          |       |      |      |      |      |      |      |      |
| 48 hour              | 29.6  | 29.4 | 31.8 | 31.4 | 29.3 | 29.4 | 29.4 | 29.1 |
| development          |       |      |      |      |      |      |      |      |
| 15 hour fade         | 53.3  | 55.6 | 56.3 | 55.5 | 50.6 | 54.5 | 56.5 | 52.0 |
| Intensity<br>decline | 23.7  | 26.2 | 24.5 | 24.1 | 21.3 | 25.1 | 27.1 | 22.9 |

It will be seen that in this instance, exceptionally, metal modification appeared to have little or no effect.

### EXAMPLE 12

This illustrates the production of a series of hydrated zirconia/hydrated silica composites in which hydrated silica predominates by a process in which hydrated zirconia is precipitated on to freshly-precipitated hydrated silica.

A master batch of hydrated silica slurry was first prepared by neutralizing sodium silicate solution (Pyramid 120) to pH 7.0 with 40% w/w sulphuric acid. The resulting hydrated silica precipitate was filtered off and washed three times with de-ionized water so as to remove substantially all water-soluble salts. The washed precipitate was then re-dispersed in de-ionized water. The silica content on a dry weight basis was checked and found to be approximately 20%.

A series of parallel experiments was then carried out in which X g of zirconyl chloride,  $ZrOCl_2 \cdot 8H_2O$  were added in each case to an amount of the above-prepared hydrated slurry equivalent to Y g silica on a dry weight basis. The pH was then adjusted to 7.0 with 10N sodium hydroxide solution, with resultant formation of a hydrated zirconia/hydrated silica composite. Z g of latex binder (Dow 675) were added. The value of Z g was selected to give an equivalent binder level in each case (15% on a dry weight basis). The experimental and test procedures from this point on were as described in Example 1. A control experiment with no zirconyl chloride solution was also carried out for comparison purposes.

The values of X, Y and Z and the zirconia content of the composite on a dry weight basis, based on the total dry weight of silica and zirconia, are set out below:

| X (g) | Y (g) | Z (g) | % $ZrO_2$ |
|-------|-------|-------|-----------|
| 0     | 25.0  | 7.5   | 0         |
| 13.4  | 22.5  | 8.3   | 18.5      |
| 26.8  | 20.0  | 9.1   | 34.0      |
| 20.2  | 8.8   | 5.0   | 46.8      |

The calender intensity and fade resistance results were as follows:

| Test<br>Conditions  | % $ZrO_2$ |      |      |      |
|---------------------|-----------|------|------|------|
|                     | 0         | 18.5 | 34.0 | 46.8 |
| 2 min. development  | 47.1      | 44.8 | 40.5 | 47.4 |
| 48 hour development | 36.6      | 36.7 | 34.5 | 40.3 |
| 15 hour fade        | 76.4      | 62.2 | 56.7 | 64.4 |
| Intensity decline   | 39.8      | 25.5 | 22.2 | 24.1 |

It will be seen that the presence of hydrated zirconia improved the initial intensity and/or fade resistance in all cases, compared with hydrated silica alone.

### EXAMPLE 13

This illustrates metal modification of a hydrated zirconia/hydrated silica composite produced by a process generally as described in Example 12, using a variety of modifying metals.

A series of parallel experiments was carried out in which 50 g of hydrated silica (20% solids content) prepared by the method described in Example 12 was added to a solution of 13.4 g of zirconyl chloride,  $ZrOCl_2 \cdot 8H_2O$  in 20 g de-ionized water. The pH was then adjusted to 7.0 using 10N sodium hydroxide solution, with resultant formation of a hydrated silica/hydrated zirconia composite. A solution of X g of a metal compound M in a small amount of de-ionized water was added and the pH was re-adjusted to 7.0. 5.4 g of latex binder (Dow 675) were added, to give a binder level of 15% on a dry weight basis. The experimental and test procedures from this point on were as described in Example 1.

The value of X and the nature of M were as set out below (it should be noted that the value of X g was chosen to give a 1.5% metal modification level on a dry weight basis, calculated as the weight of metal oxide in relation to the total weight of zirconia, silica and metal oxide).

| X (g) | M                  |
|-------|--------------------|
| 1.76  | Ferrous sulphate   |
| 1.78  | Cobalt sulphate    |
| 1.78  | Nickel sulphate    |
| 1.58  | Copper sulphate    |
| 0.86  | Calcium sulphate   |
| 1.56  | Magnesium sulphate |
| 1.82  | Zinc sulphate      |

The calendar intensity and fade resistance results obtained were as follows:

| Test<br>Conditions  | metal |      |      |      |      |      |      |
|---------------------|-------|------|------|------|------|------|------|
|                     | Fe    | Co   | Ni   | Cu   | Ca   | Mg   | Zn   |
| 2 min. development  | 38.6  | 42.7 | 42.5 | 38.8 | 39.6 | 42.6 | 47.6 |
| 48 hour development | 33.5  | 38.6 | 36.8 | 34.6 | 34.8 | 37.1 | 43.1 |
| 15 hour fade        | 57.9  | 55.1 | 52.9 | 54.3 | 58.5 | 58.3 | 60.1 |
| Intensity decline   | 24.4  | 16.5 | 16.1 | 19.7 | 23.7 | 21.2 | 17.0 |

### EXAMPLE 14

This illustrates the production of a series of hydrated zirconia/hydrated silica composites by a process in which the hydrated zirconia and hydrated silica are precipitated from solution together.

Z g of 30% w/w solution of zirconyl chloride,  $ZrOCl_2 \cdot 8H_2O$  were slowly added to 5 g of 30% w/w solution of sodium silicate (3.2:1  $SiO_2:Na_2O$ ) with stirring and the pH of the resulting mixture was adjusted to 7.0 using 20% w/w sulphuric acid. This resulted in precipitation of a hydrated zirconia/hydrated silica composite. The precipitate was filtered off, washed twice with de-ionized water so as to remove soluble salts, and re-dispersed in de-ionized water. This dispersion was then ball-milled to give a mean particle size of approximately 4  $\mu m$  (as measured by a Coulter Counter). 17.65 g of latex binder (Dow 675) were added which gave a 15% latex content on a dry weight basis. The experimental and test procedures from this point on

were as described in Example 1, except that different test papers were used, namely Paper D which utilised CVL as the sole colour former, Paper E which utilised a slow developing blue colour former (Pergascript Blue BP 558 supplied by Ciba-Geigy) as the sole colour former, and Paper F which utilised a commercially used blend of colour formers including CVL and a slow-developing blue colour former.

The values of Z and S and the zirconia content of the composite on a dry weight basis, based on the total dry weight of zirconia and silica were as follows:

| Z (g)  | S (g)  | % ZrO <sub>2</sub> |
|--------|--------|--------------------|
| 87.26  | 200.00 | 20                 |
| 174.53 | 150.00 | 40                 |
| 261.79 | 100.00 | 60                 |
| 349.05 | 50.00  | 80                 |

The calender intensity and fade resistance results were as follows:

| Paper D             |            | % ZrO <sub>2</sub> |      |      |    |
|---------------------|------------|--------------------|------|------|----|
| Test                | Conditions | 20                 | 40   | 60   | 80 |
| 2 min. development  | 57.2       | 53.5               | 50.3 | 50.4 |    |
| 48 hour development | 46.1       | 46.1               | 46.6 | 47.6 |    |
| 15 hour fade        | 94.6       | 93.7               | 82.8 | 82.8 |    |
| Intensity decline   | 48.5       | 47.6               | 36.2 | 39.9 |    |

| Paper E             |            | % ZrO <sub>2</sub> |      |      |    |
|---------------------|------------|--------------------|------|------|----|
| Test                | Conditions | 20                 | 40   | 60   | 80 |
| 2 min. development  | —          | —                  | —    | —    |    |
| 48 hour development | 60.5       | 64.0               | 60.7 | 62.9 |    |
| 15 hour fade        | 66.4       | 63.8               | 65.0 | 77.0 |    |
| Intensity decline   | 5.9        | —0.2               | 4.3  | 14.1 |    |

| Paper F             |            | % ZrO <sub>2</sub> |      |      |    |
|---------------------|------------|--------------------|------|------|----|
| Test                | Conditions | 20                 | 40   | 60   | 80 |
| 2 min. development  | 46.4       | 42.4               | 41.4 | 39.8 |    |
| 48 hour development | 36.1       | 35.5               | 37.0 | 37.6 |    |
| 15 hour fade        | 76.9       | 73.7               | 61.6 | 64.7 |    |
| Intensity decline   | 40.8       | 38.2               | 24.6 | 27.1 |    |

### EXAMPLE 15

This illustrates the production of a series of hydrated zirconia/hydrated silica/hydrated alumina composites by a process in which the hydrated zirconia and hydrated silica are first precipitated from solution together and hydrated alumina is then precipitated on to the hydrated zirconia/hydrated silica composite so formed.

The procedure was as described in Example 14 except that after precipitation of the hydrated zirconia/hydrated silica composite, A g of 40% w/w solution of aluminium sulphate, Al<sub>2</sub>(SO<sub>4</sub>)<sub>3</sub>.16H<sub>2</sub>O were added and the pH was readjusted to 7.0 using 10N sodium hydroxide solution. The precipitate was then filtered off and the subsequent procedure was as in Example 14, except that no tests were made using Paper E, except for Composition No. 7 (see below).

The values of Z, S and A, and the relative proportions of zirconia, silica and alumina in the composite on

a dry weight basis, based on the total dry weight of zirconia, silica and alumina were as follows:

| 5 | Composition | Z (g)  | S (g)  | A (g)  | ZrO <sub>2</sub> :SiO <sub>2</sub> :Al <sub>2</sub> O <sub>3</sub> (%) |
|---|-------------|--------|--------|--------|------------------------------------------------------------------------|
| 1 | 1           | 87.26  | 150.00 | 154.41 | 20:60:20                                                               |
| 2 | 2           | 87.26  | 100.00 | 308.82 | 20:40:40                                                               |
| 3 | 3           | 87.26  | 50.00  | 463.23 | 20:20:60                                                               |
| 4 | 4           | 174.53 | 100.00 | 154.41 | 40:40:20                                                               |
| 5 | 5           | 174.53 | 50.00  | 308.82 | 40:20:40                                                               |
| 6 | 6           | 261.79 | 50.00  | 154.41 | 60:20:20                                                               |
| 7 | 7           | 145.44 | 83.33  | 257.35 | 33.3:33.3:33.3                                                         |

The calender intensity and fade resistance results were as follows:

| 15                  | Paper D         |      |      |      |      |      |      |
|---------------------|-----------------|------|------|------|------|------|------|
| Test                | Composition No. |      |      |      |      |      |      |
| Conditions          | 1               | 2    | 3    | 4    | 5    | 6    | 7    |
| 2 min. development  | 54.3            | 51.8 | 51.8 | 52.5 | 51.4 | 51.8 | 50.3 |
| 48 hour development | 45.0            | 45.9 | 44.3 | 47.0 | 46.4 | 44.9 | 46.3 |
| 15 hour fade        | 75.5            | 69.0 | 68.8 | 77.5 | 70.7 | 73.9 | 82.4 |
| Intensity decline   | 30.5            | 24.1 | 24.5 | 30.5 | 24.3 | 29.0 | 36.1 |

For Paper E and the coated paper made using Composition No. 7, the results were:

|    |                     |      |
|----|---------------------|------|
| 30 | 48 hour development | 59.6 |
|    | 15 hour fade        | 66.8 |
|    | Intensity decline   | 7.2  |

(No measurement was made after 2 min. development).

| 35                  | Paper F         |      |      |      |      |      |      |
|---------------------|-----------------|------|------|------|------|------|------|
| Test                | Composition No. |      |      |      |      |      |      |
| Conditions          | 1               | 2    | 3    | 4    | 5    | 6    | 7    |
| 2 min. development  | 42.4            | 41.6 | 39.9 | 38.0 | 37.8 | 39.1 | 38.9 |
| 48 hour development | 34.0            | 35.5 | 34.0 | 33.9 | 34.5 | 33.6 | 34.9 |
| 15 hour fade        | 47.0            | 49.7 | 51.9 | 55.6 | 56.9 | 57.6 | 61.9 |
| Intensity decline   | 13.0            | 14.2 | 17.9 | 21.7 | 22.4 | 24.0 | 27.0 |

### EXAMPLE 16

This illustrates the production of a series of hydrated zirconia/hydrated silica/hydrated alumina composites by a process in which hydrated alumina and hydrated silica are first precipitated from solution together and hydrated zirconia is then precipitated on to the hydrated zirconia/hydrated silica composite so formed.

A g of 40% w/w solution of aluminium sulphate Al<sub>2</sub>(SO<sub>4</sub>)<sub>3</sub>.16H<sub>2</sub>O were slowly added to S g of 30% w/w solution of sodium silicate (3.2:1 SiO<sub>2</sub>:Na<sub>2</sub>O), with stirring, and the pH of the resulting mixture was adjusted to 7.0 using 20% w/w sulphuric acid. This resulted in precipitation of a hydrated silica/hydrated alumina composite. Z g of 30% w/w solution of zirconyl chloride ZrOCl<sub>2</sub>.8H<sub>2</sub>O were then added and the pH was readjusted to 7.0 using 10N sodium hydroxide solution, with resultant precipitation of hydrated zirconia. The composite precipitate was filtered off and the procedure from this point was as in Example 15.

The values of Z, S and A, and the proportions of zirconia:silica:alumina in the composite on a dry weight basis were the same as in Example 15.

The calender intensity and fade resistance results were as follows:

| Test<br>Conditions  | Paper D         |      |      |      |      |      |      |
|---------------------|-----------------|------|------|------|------|------|------|
|                     | Composition No. |      |      |      |      |      |      |
|                     | 1               | 2    | 3    | 4    | 5    | 6    | 7    |
| 2 min. development  | 48.8            | 48.7 | 48.3 | 49.3 | 49.0 | 47.4 | 51.8 |
| 48 hour development | 46.5            | 45.6 | 44.3 | 45.4 | 44.4 | 44.9 | 49.2 |
| 15 hour fade        | 78.6            | 72.3 | 70.2 | 77.2 | 75.3 | 74.7 | 85.2 |
| Intensity decline   | 32.1            | 26.1 | 25.9 | 31.8 | 30.9 | 29.8 | 36.0 |

| Test<br>Conditions  | Paper E         |      |      |      |      |      |      |
|---------------------|-----------------|------|------|------|------|------|------|
|                     | Composition No. |      |      |      |      |      |      |
|                     | 1               | 2    | 3    | 4    | 5    | 6    | 7    |
| 2 min. development  | —               | —    | —    | —    | —    | —    | —    |
| 48 hour development | 62.1            | 60.4 | 66.5 | 63.9 | 60.7 | 63.5 | 62.7 |
| 15 hour fade        | 60.9            | 60.9 | 66.6 | 63.1 | 63.6 | 68.6 | 71.9 |
| Intensity decline   | —1.2            | 0.5  | 0.1  | —0.8 | 2.9  | 5.1  | 9.2  |

| Test<br>Conditions  | Paper F         |      |      |      |      |      |      |
|---------------------|-----------------|------|------|------|------|------|------|
|                     | Composition No. |      |      |      |      |      |      |
|                     | 1               | 2    | 3    | 4    | 5    | 6    | 7    |
| 2 min. development  | 37.1            | 37.3 | 37.2 | 38.8 | 35.3 | 37.4 | 40.7 |
| 48 hour development | 34.1            | 33.6 | 33.7 | 34.8 | 32.2 | 33.8 | 35.8 |
| 15 hour fade        | 53.2            | 49.6 | 52.1 | 56.9 | 50.9 | 57.5 | 66.9 |
| Intensity decline   | 19.1            | 16.0 | 18.4 | 22.1 | 18.7 | 13.7 | 31.1 |

### EXAMPLE 17

This illustrates the production of a series of hydrated zirconia/hydrated alumina composites by a process in which hydrated zirconia and hydrated alumina are precipitated from solution together.

A g of 40% w/w solution of aluminium sulphate,  $\text{Al}_2(\text{SO}_4)_3 \cdot 16\text{H}_2\text{O}$  were added to Z g of 30% w/w solution of zirconyl chloride  $\text{ZrOCl}_2 \cdot 8\text{H}_2\text{O}$  with stirring, and the pH of the resulting mixture was adjusted to 7.0 using 10N sodium hydroxide solution. This resulted in precipitation of a hydrated zirconia/hydrated alumina composite. The procedure from this point on was as in Example 14.

The values of A and Z and the zirconia content of the composite on a dry weight basis, based on the total dry weight of zirconia and silica were as follows:

| A (g)  | Z (g)  | % $\text{ZrO}_2$ |
|--------|--------|------------------|
| 617.64 | 87.26  | 20               |
| 463.23 | 174.53 | 40               |
| 308.82 | 261.79 | 60               |
| 154.41 | 349.05 | 80               |

The calendar intensity and face resistance results were as follows:

| Test<br>Conditions | Paper D          |      |      |      |
|--------------------|------------------|------|------|------|
|                    | % $\text{ZrO}_2$ |      |      |      |
|                    | 20               | 40   | 60   | 80   |
| 2 min. development | 53.4             | 52.9 | 51.2 | 48.2 |

-continued

| Test<br>Conditions  | Paper D          |      |      |      |
|---------------------|------------------|------|------|------|
|                     | % $\text{ZrO}_2$ |      |      |      |
|                     | 20               | 40   | 60   | 80   |
| 48 hour development | 46.5             | 45.5 | 45.4 | 44.3 |
| 15 hour fade        | 89.1             | 83.7 | 82.7 | 85.9 |
| Intensity decline   | 42.6             | 38.2 | 37.3 | 41.6 |

| Test<br>Conditions  | Paper E          |    |      |      |
|---------------------|------------------|----|------|------|
|                     | % $\text{ZrO}_2$ |    |      |      |
|                     | 20               | 40 | 60   | 80   |
| 2 min. development  | —                | —  | —    | —    |
| 48 hour development | —                | —  | 62.4 | 63.3 |
| 15 hour fade        | —                | —  | 53.1 | 85.1 |
| Intensity decline   | —                | —  | 20.7 | 24.8 |

| Test<br>Conditions  | Paper F          |      |      |      |
|---------------------|------------------|------|------|------|
|                     | % $\text{ZrO}_2$ |      |      |      |
|                     | 20               | 40   | 60   | 80   |
| 2 min development   | 40.8             | 39.4 | 37.5 | 37.3 |
| 48 hour development | 33.8             | 34.3 | 33.4 | 33.6 |
| 15 hour fade        | 70.2             | 66.3 | 65.7 | 77.2 |
| Intensity decline   | 36.4             | 32.0 | 32.3 | 43.6 |

### EXAMPLE 18

This illustrates the production of two hydrated zirconia/hydrated silica/hydrated alumina composites by a process in which the hydrated zirconia and hydrated alumina are first precipitated from solution together and hydrated silica is then precipitated on to the hydrated zirconia/hydrated alumina composite so formed.

The procedure was as described in Example 17 above except that after precipitation of the hydrated zirconia/hydrated alumina composite, S g of a solution of 30% w/w sodium silicate (3.2:1  $\text{SiO}_2:\text{Na}_2\text{O}$ ) were added and the pH was re-adjusted to 7.0 using 20% w/w sulphuric acid. The precipitate was then filtered off and the subsequent procedure was as in Example 14.

The values of Z, S and A, and the proportions of zirconia:silica:alumina in the composite on a dry weight basis, based on the total dry weight of zirconia, silica and alumina were as follows:

| Z (g)  | S (g)  | A (g)  | $\text{ZrO}_2:\text{SiO}_2:\text{Al}_2\text{O}_3$ (%) |
|--------|--------|--------|-------------------------------------------------------|
| 145.44 | 83.33  | 257.35 | 33:33:33                                              |
| 174.53 | 100.00 | 154.41 | 40:40:20                                              |

The above procedure was then repeated in a second run, and the results of the calender intensity and fade resistance tests were as follows:

| Test<br>Conditions  | Run No. |      |         |      |
|---------------------|---------|------|---------|------|
|                     | Paper D |      | Paper F |      |
|                     | 1       | 2    | 1       | 2    |
| 2 min. development  | 54.7    | 53.9 | 43.7    | 43.4 |
| 48 hour development | 48.0    | 51.0 | 36.3    | 36.3 |
| 15 hour fade        | 80.7    | 80.9 | 57.1    | 57.5 |
| Intensity decline   | 32.7    | 29.9 | 20.8    | 21.2 |

No testing was done in this instance with Paper E.

No testing was done in this instance with Paper E.

## EXAMPLE 19

This illustrates the production of a hydrated zirconia/hydrated silica/hydrated alumina composite by a process in which hydrated silica is first precipitated, followed by hydrated zirconia, followed by hydrated alumina.

20% w/w sulphuric acid was added to 83.33 g of a 30% w/w solution of sodium silicate (3.2:1 SiO<sub>2</sub>:Na<sub>2</sub>O) until the pH was 7.0, by which time hydrated silica had been precipitated. 145.44 g of 30% w/w solution of zirconyl chloride ZrOCl<sub>2</sub>.8H<sub>2</sub>O were added, and the pH was readjusted to 7.0 by the addition of 10N sodium hydroxide solution, with resultant precipitation of hydrated zirconia. 257.35 g of 40% w/w solution of aluminium sulphate, Al<sub>2</sub>(SO<sub>4</sub>)<sub>3</sub>.16H<sub>2</sub>O were added and the pH was re-adjusted to 7.0 with 10N sodium hydroxide solution, with resultant precipitation of hydrated alumina. The resultant composite precipitate was filtered off and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 54.0       | —       | 40.4    |
| 48 hour development | 47.8       | 60.2    | 35.8    |
| 15 hour fade        | 74.4       | 64.7    | 56.8    |
| Intensity decline   | 26.6       | 4.5     | 21.0    |

## EXAMPLE 20

This illustrates the production of a hydrated zirconia/hydrated silica/hydrated alumina composite by a process in which hydrated zirconia is first precipitated, followed by hydrated silica, followed by hydrated alumina.

10N sodium hydroxide solution was added to 145.44 g of 30% w/w solution of zirconyl chloride, ZrOCl<sub>2</sub>.8H<sub>2</sub>O until the pH was 7.0 by which time hydrated zirconia had been precipitated. 83.33 g of a 30% w/w solution of sodium silicate (3.2:1 SiO<sub>2</sub>:Na<sub>2</sub>O) were added and the pH was readjusted to 7.0 with 20% w/w sulphuric acid, with resultant precipitation of hydrated silica. 257.35 g of 40% w/w solution of aluminium sulphate, Al<sub>2</sub>(SO<sub>4</sub>)<sub>3</sub>.16H<sub>2</sub>O were added and the pH was re-adjusted to 7.0 with 10N sodium hydroxide solution, with resultant precipitation of hydrated alumina. The resultant composite precipitate was filtered off and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 52.8       | —       | 40.9    |
| 48 hour development | 46.2       | 59.3    | 33.9    |
| 15 hour fade        | 74.6       | 63.7    | 54.9    |
| Intensity decline   | 28.4       | 4.4     | 21.0    |

## EXAMPLE 21

This illustrates the production of a hydrated zirconia/hydrated silica/hydrated alumina composite by a process in which hydrated zirconia is first precipitated,

followed by hydrated alumina, followed by hydrated silica.

10N sodium hydroxide solution was added to 145.44 g of 30% w/w solution of zirconyl chloride ZrOCl<sub>2</sub>.8H<sub>2</sub>O until the pH was 7.0, by which time hydrated zirconia had been precipitated. 257.35 g of 40% w/w solution of aluminium sulphate, Al<sub>2</sub>(SO<sub>4</sub>)<sub>3</sub>.16H<sub>2</sub>O were added and the pH was re-adjusted to 7.0 with 10N sodium hydroxide solution, with resultant precipitation of hydrated alumina. 83.33 g of a 30% w/w solution of sodium silicate (3.2:1 SiO<sub>2</sub>:Na<sub>2</sub>O) were then added and the pH was re-adjusted to 7.0 with 20% w/w sulphuric acid, with resultant precipitation of hydrated silica. The composite precipitate was filtered off and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 53.0       | —       | 41.4    |
| 48 hour development | 47.2       | 61.5    | 36.4    |
| 15 hour fade        | 73.6       | 63.6    | 55.4    |
| Intensity decline   | 26.4       | 2.1     | 19.0    |

## EXAMPLE 22

This illustrates the production of a hydrated zirconia/hydrated silica/hydrated alumina composite by a process in which hydrated alumina is first precipitated, followed by hydrated zirconia, followed by hydrated silica.

10N sodium hydroxide solution was added to 257.35 g of 40% w/w solution of aluminium sulphate, Al<sub>2</sub>(SO<sub>4</sub>)<sub>3</sub>.16H<sub>2</sub>O until the pH was 7.0 by which time hydrated alumina had been precipitated. 145.44 g of 30% w/w solution of zirconyl chloride ZrOCl<sub>2</sub>.8H<sub>2</sub>O were added, and the pH was re-adjusted to 7.0 by the addition of 10N sodium hydroxide solution, with resultant precipitation of hydrated zirconia. 83.33 g of a 30% w/w solution of sodium silicate (3.2:1 SiO<sub>2</sub>:Na<sub>2</sub>O) were then added and the pH was re-adjusted to 7.0 using 20% w/w sulphuric acid, with resultant precipitation of hydrated silica. The composite precipitate was filtered off and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 53.0       | —       | 41.3    |
| 48 hour development | 45.5       | 63.9    | 34.7    |
| 15 hour fade        | 63.1       | 65.7    | 44.7    |
| Intensity decline   | 17.6       | 1.8     | 10.0    |

## EXAMPLE 23

This illustrates the production of a hydrated zirconia/hydrated silica/hydrated alumina composite by a process in which hydrated silica is first precipitated, followed by hydrated alumina, followed by hydrated zirconia.

20% w/w sulphuric acid was added to 83.33 g of 30% w/w sodium silicate solution (3.2:1 SiO<sub>2</sub>:Na<sub>2</sub>O) until the pH was 7.0, by which time hydrated silica had been precipitated. 257.35 g of 40% w/w solution of

aluminium sulphate,  $Al_2(SO_4)_3 \cdot 16H_2O$  were added and the pH was re-adjusted to 7.0 with 10N sodium hydroxide solution, with resultant precipitation of hydrated alumina. 145.44 g of 30% w/w solution of zirconyl chloride  $ZrOCl_2 \cdot 8H_2O$  were added, and the pH was re-adjusted to 7.0 by the addition of 10N sodium hydroxide solution, with resultant precipitation of hydrated zirconia. The composite precipitate was filtered off and the procedure from this point was as in Example 14.

The calender intensity and fade resistance results were as follows:

| Test Conditions     | Test Paper |         |         |
|---------------------|------------|---------|---------|
|                     | Paper D    | Paper E | Paper F |
| 2 min. development  | 55.6       | —       | 41.7    |
| 48 hour development | 51.2       | 64.1    | 37.6    |
| 15 hour fade        | 78.4       | 68.2    | 57.8    |
| Intensity decline   | 27.2       | 4.1     | 20.2    |

#### EXAMPLE 24

This illustrates the production of a hydrated zirconia/hydrated silica/hydrated alumina composite by a process in which hydrated alumina is first precipitated, followed by hydrated silica, followed by hydrated zirconia.

10N sodium hydroxide solution was added to 257.35 g of 40% w/w solution of aluminium sulphate,  $Al_2(SO_4)_3 \cdot 16H_2O$  until the pH was 7.0 by which time hydrated alumina had been precipitated. 83.33 g of 30% w/w sodium silicate solution (3.2:1  $SiO_2:Na_2O$ ) were then added and the pH was re-adjusted to 7.0 using 20% w/w sulphuric acid, with resultant precipitation of hydrated silica. 145.44 g of 30% w/w solution of zirconyl chloride  $ZrOCl_2 \cdot 8H_2O$  were added, and the pH was re-adjusted to 7.0 by the addition of 10N sodium hydroxide solution with resultant precipitation of hydrated zirconia. The composite precipitate was filtered off and the procedure from this point was as in Example 14.

The calender intensity and fade resistance results were as follows:

| Test Conditions     | Test Paper |         |         |
|---------------------|------------|---------|---------|
|                     | Paper D    | Paper E | Paper F |
| 2 min. development  | 57.4       | —       | 37.5    |
| 48 hour development | 46.2       | 63.3    | 34.0    |
| 15 hour fade        | 73.9       | 70.6    | 56.3    |
| Intensity decline   | 27.7       | 7.3     | 22.3    |

#### EXAMPLE 25

This illustrates the preparation of a hydrated zirconia/hydrated alumina composite by a process in which hydrated zirconia and hydrated alumina, both in freshly-precipitated form, are admixed.

10N sodium hydroxide solution was added to 218.16 g of 30% w/w solution of zirconyl chloride,  $ZrOCl_2 \cdot 8H_2O$  until the pH was 7.0, with resultant precipitation of hydrated zirconia.

10N sodium hydroxide solution was also added to 386.03 g of 40% w/w solution of aluminium sulphate,  $Al_2(SO_4)_3 \cdot 16H_2O$  until the pH was 7.0, with resultant precipitation of hydrated alumina.

The precipitates from the above were each filtered off and washed twice with de-ionized water before

being redispersed in de-ionized water. The dispersions were each ball-milled until the particle size of the composite was approximately 4  $\mu m$  (as measured using a Coulter Counter), after which they were combined, and 17.65 g latex binder (Dow 675) were added, so as to give a 15% latex content on a dry weight basis. The procedure from this point on was as in Example 14.

The calender intensity and fade resistance results were as follows:

| Test Conditions     | Test Paper |         |         |
|---------------------|------------|---------|---------|
|                     | Paper D    | Paper E | Paper F |
| 2 min. development  | 50.8       | —       | 38.5    |
| 48 hour development | 45.4       | 73.9    | 32.6    |
| 15 hour fade        | 74.6       | 82.1    | 56.1    |
| Intensity decline   | 29.2       | 8.2     | 23.5    |

#### EXAMPLE 26

This illustrates the preparation of a hydrated zirconia/hydrated silica composite by a process in which hydrated zirconia and hydrated silica, both in freshly-precipitated form, are admixed.

10N sodium hydroxide solution was added to 218.16 g of 30% w/w solution of zirconyl chloride,  $ZrOCl_2 \cdot 8H_2O$  until the pH was 7.0, with resultant precipitation of hydrated zirconia.

20% w/w sulphuric acid was also added to 125.00 g of 30% w/w sodium silicate solution (3.2:1  $SiO_2:Na_2O$ ) until the pH was 7.0, with resultant precipitation of hydrated silica.

The precipitates from the above were each filtered off and washed twice with de-ionized water before being redispersed in de-ionized water. The dispersions were each ball-milled until the particle size of the composite was approximately 4  $\mu m$  (as measured using a Coulter Counter), after which they were combined, and 17.63 g latex binder (Dow 675) were added, so as to give a 15% latex content on a dry weight basis. The procedure from this point on was as in Example 14.

The calender intensity and fade resistance results were as follows:

| Test Conditions     | Test Paper |         |         |
|---------------------|------------|---------|---------|
|                     | Paper D    | Paper E | Paper F |
| 2 min. development  | 56.1       | —       | 42.7    |
| 48 hour development | 51.5       | 71.6    | 37.8    |
| 15 hour fade        | 94.3       | 69.4    | 72.9    |
| Intensity decline   | 42.8       | —2.2    | 35.1    |

#### EXAMPLE 27

This illustrates the preparation of a hydrated zirconia/hydrated silica/hydrated alumina composite by a process in which hydrated zirconia, hydrated silica and hydrated alumina, all in freshly-precipitated form, are admixed.

10N sodium hydroxide solution was added to 145.44 g of 30% w/w solution of zirconyl chloride,  $ZrOCl_2 \cdot 8H_2O$  until the pH was 7.0, with resultant precipitation of hydrated zirconia.

10N sodium hydroxide solution was also added to 257.35 g of 40% w/w solution of aluminium sulphate,  $Al_2(SO_4)_3 \cdot 16H_2O$  until the pH was 7.0, with resultant precipitation of hydrated alumina. 20% w/w sulphuric acid was also added to 83.33 g of 30% w/w sodium

silicate solution (3.2:1 SiO<sub>2</sub>:Na<sub>2</sub>O) until the pH was 7.0, with resultant precipitation of hydrated silica.

The precipitates from the above were each filtered off and washed twice with de-ionized water before being redispersed in de-ionized water. The dispersions were each ball-milled until the particle size of the composite was approximately 4  $\mu\text{m}$  (as measured using a Coulter Counter), after which they were combined, and 17.65 g latex binder (Dow 675) were added, so as to give a 15% latex content on a dry weight basis. The procedure from this point on was as in Example 14.

The calender intensity and fade resistance results were as follows:

| Test<br>Conditions   | Test Paper |         |         |
|----------------------|------------|---------|---------|
|                      | Paper D    | Paper E | Paper F |
| 2 min. development   | 53.4       | —       | 40.8    |
| 48 hours development | 49.2       | 64.8    | 35.4    |
| 15 hours fade        | 66.7       | 66.2    | 50.1    |
| Intensity decline    | 17.5       | 1.4     | 14.7    |

### EXAMPLE 28

This illustrates the production of a hydrated zirconia/hydrated silica/hydrated alumina composite by a process in which hydrated silica and hydrated alumina are precipitated together on to previously-precipitated hydrated zirconia.

10N sodium hydroxide solution was added to 145.44 g of 30% w/w solution of zirconyl chloride, ZrOCl<sub>2</sub>.8-H<sub>2</sub>O until the pH was 7.0, with resultant precipitation of hydrated zirconia. 83.33 g of a 30% w/w solution of sodium silicate (3.2:1 SiO<sub>2</sub>:Na<sub>2</sub>O) were added, followed slowly by 257.35 g of 40% w/w solution of aluminium sulphate, Al<sub>2</sub>(SO<sub>4</sub>)<sub>3</sub>.16H<sub>2</sub>O and the pH of the resulting mixture was re-adjusted to 7.0, with 10N sodium hydroxide solution, with resultant precipitation of hydrated silica and hydrated alumina on to the hydrated zirconia. The composite precipitate was filtered off, and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 52.3       | —       | 37.9    |
| 48 hour development | 48.0       | 65.0    | 35.2    |
| 15 hour fade        | 65.4       | 69.3    | 48.5    |
| Intensity decline   | 17.4       | 4.3     | 13.3    |

### EXAMPLE 29

This illustrates the production of a hydrated zirconia/hydrated silica/hydrated alumina composite by a process in which hydrated zirconia and hydrated silica are precipitated together on to previously-precipitated hydrated alumina.

10N sodium hydroxide solution was added to 257.35 g of 40% w/w solution of aluminium sulphate, Al<sub>2</sub>(SO<sub>4</sub>)<sub>3</sub>.16H<sub>2</sub>O until the pH was 7.0, with resultant precipitation of hydrated alumina. 83.33 g of a 30% w/w solution of sodium silicate (3.2:1 SiO<sub>2</sub>:Na<sub>2</sub>O) were added, followed slowly by 145.44 g of 30% w/w solution of zirconyl chloride, ZrOCl<sub>2</sub>.8H<sub>2</sub>O and the pH of the resulting mixture was re-adjusted to 7.0 with 10N sodium hydroxide solution, with resultant precipitation of hydrated zirconia and hydrated silica on to the hydrated alumina.

hydrated alumina. The composite precipitate was filtered off, and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 51.6       | —       | 39.7    |
| 48 hour development | 46.5       | 68.6    | 34.7    |
| 15 hour fade        | 72.5       | 74.6    | 53.4    |
| Intensity decline   | 26.0       | 6.0     | 18.7    |

15

### EXAMPLE 30

This illustrates the production of a hydrated zirconia/hydrated silica/hydrated alumina composite by a process in which hydrated zirconia and hydrated alumina are precipitated together on to previously-precipitated hydrated silica.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 860

-continued

| Test<br>Conditions  | Test Paper |         |         |
|---------------------|------------|---------|---------|
|                     | Paper D    | Paper E | Paper F |
| 48 hour development | 46.2       | 79.7    | 34.3    |
| 15 hour fade        | 85.8       | 91.0    | 65.1    |
| Intensity decline   | 39.6       | 11.3    | 30.8    |

## EXAMPLE 32

This illustrates the production of a hydrated zirconia/hydrated silica/hydrated alumina composite by a process in which hydrated silica and hydrated alumina are precipitated together on to previously-precipitated hydrated zirconia, but which differs from Example 28 in that sodium aluminate is used in place of aluminium sulphate.

10N sodium hydroxide solution was added to 145.44 g of 30% w/w solution of zirconyl chloride,  $ZrOCl_2 \cdot 8 \cdot H_2O$  until the pH was 7.0, with resultant precipitation of hydrated zirconia. 83.33 g of 30% w/w sodium silicate solution (3.2:1  $SiO_2:Na_2O$ ) were added, followed by 66.12 g of 40% w/w sodium aluminate solution, and the pH of the resulting mixture was re-adjusted to 7.0 with 10N sodium hydrated solution, with resultant precipitation of hydrated silica and hydrated alumina on to the hydrated zirconia. The composite precipitate was filtered off, and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 50.2       | —       | 39.0    |
| 48 hour development | 46.3       | 63.8    | 35.0    |
| 15 hour fade        | 75.7       | 68.1    | 54.9    |
| Intensity decline   | 29.4       | -4.3    | 19.9    |

## EXAMPLE 33

This illustrates the production of a hydrated zirconia/hydrated silica/hydrated alumina composite by a process in which hydrated silica and hydrated alumina are precipitated together on to previously-precipitated hydrated zirconia, but which differs from Example 28 in that zirconium sulphate is used in place of zirconyl chloride.

10N sodium hydroxide solution was added to 92.59 g of 30% w/w solution of zirconium sulphate,  $Zr(SO_4)_2 \cdot H_2O$  until the pH was 7.0, with resultant precipitation of hydrated zirconia. 83.33 g of 30% w/w sodium silicate solution (3.2:1  $SiO_2:Na_2O$ ) were added, followed slowly by 257.35 g of 40% w/w solution of aluminium sulphate,  $Al_2(SO_4)_3 \cdot 16H_2O$  and the pH of the resulting mixture was re-adjusted to 7.0 with 10N sodium hydroxide solution, with resultant precipitation of hydrated silica and hydrated alumina on to the hydrated zirconia. The composite precipitate was filtered off, and the procedure from this point was as in Example 14.

The calender intensity and fade resistance results were as follows:

| Test<br>Conditions | Test Paper |         |         |
|--------------------|------------|---------|---------|
|                    | Paper D    | Paper E | Paper F |
| 2 min. development | 52.5       | —       | 42.1    |

-continued

| Test<br>Conditions  | Test Paper |         |         |
|---------------------|------------|---------|---------|
|                     | Paper D    | Paper E | Paper F |
| 48 hour development | 45.2       | 64.3    | 33.9    |
| 15 hour fade        | 74.9       | 70.4    | 55.1    |
| Intensity decline   | 29.7       | 6.1     | 21.2    |

## EXAMPLE 34

This illustrates the production of a hydrated zirconia/hydrated silica/hydrated alumina composite by a process in which hydrated silica and hydrated alumina are precipitated together on to previously-precipitated hydrated zirconia, but which differs from Example 28 in that zirconium nitrate is used in place of zirconyl chloride.

10N sodium hydroxide solution was added to 97.11 g of 30% w/w solution of zirconium nitrate (anhydrous) until the pH was 7.0, with resultant precipitation of hydrated zirconia. 83.33 g of 30% w/w sodium silicate solution (3.2:1  $SiO_2:Na_2O$ ) were added, followed slowly by 257.35 g of 40% w/w solution of aluminium sulphate,  $Al_2(SO_4)_3 \cdot 16H_2O$ , and the pH of the resulting mixture was re-adjusted to 7.0 with 10N sodium hydroxide solution, with resultant precipitation of hydrated silica and hydrated alumina on to the hydrated zirconia. The composite precipitate was filtered off, and the procedure from this point was as in Example 14.

The calender intensity and fade resistance results were as follows:

| Test<br>Conditions  | Test Paper |         |         |
|---------------------|------------|---------|---------|
|                     | Paper D    | Paper E | Paper F |
| 2 min. development  | 54.3       | —       | 46.6    |
| 48 hour development | 46.6       | 64.7    | 35.9    |
| 15 hour fade        | 72.4       | 69.9    | 55.7    |
| Intensity decline   | 25.8       | 5.2     | 19.2    |

## EXAMPLE 35

This demonstrates the suitability of a typical example of a colour former according to the invention for use in heat-sensitive record material.

20 g of a washed and dried hydrated zirconia/hydrated alumina/hydrated zirconia composite prepared by the method of Example 1 (Run No. 1) were mixed with 48 g of stearamide wax and ground in a pestle and mortar. 45 g of de-ionized water and 60 g of 10% w/w poly(vinyl alcohol) solution (that supplied as "Gohsenol GL05" by Nippon Gohsei of Japan) were added and the mixture was ball-milled overnight. A further 95 g of 10% w/w poly(vinyl alcohol) solution were then added, together with 32 g de-ionized water.

In a separate procedure, 22 g of a black colour former (2'-anilino-6'-diethylamino-3'-methylfluoran), were mixed with 42 g de-ionized water and 100 g of 10% w/w poly(vinyl alcohol) solution, and the mixture was ball-milled overnight.

The suspensions resulting from the above procedures were then mixed and coated on to paper by means of a laboratory Meyer bar coater at a nominal coat weight of 8  $gm^{-2}$ . The paper was then dried.

On subjecting the coated surface to heat, a black colouration was obtained.

I claim:

1. Record material carrying a colour developer composition which comprises a particulate composite having as components hydrated zirconia and at least one of hydrated silica and hydrated alumina.

2. Record material as claimed in claim 1, characterized in that at least one of the components of the com-

posite is present in a greater proportion in a surface region of the composite than elsewhere.

3. Record material as claimed in claim 2, characterized in that the composite is modified by the presence of a compound or ions of one or more multivalent metals.

4. Record material as claimed in claim 1 characterized in that the composite is modified by the presence of a compound or ions of one or more multivalent metals.

\* \* \* \* \*

10

15

20

25

30

35

40

45

50

55

60

65